

# UNITED STATES PATENT OFFICE.

ALBERT C. HOLZAPFEL, OF NEW YORK, N. Y.

## FLOOR-COVERING.

1,353,371.

Specification of Letters Patent. Patented Nov. 9, 1920.

No Drawing.

Application filed December 28, 1919. Serial No. 346,920.

To all whom it may concern:

Be it known that I, ALBERT C. HOLZAPFEL, a subject of the King of England, residing at New York, in the county of New York and State of New York, have invented certain new and useful Improvements in Floor-Coverings, of which the following is a specification.

This invention relates to floor coverings of the character commonly known as linoleum, and has particular reference to certain improvements therein, whereby a satisfactory, serviceable and durable floor covering of this character can be produced at materially less expense than linoleums now in use.

In the present invention, I employ certain organic waxes or pitches derived from the treatment of oils and fats, such as stearin pitch, palm oil pitch and the like, in place of the linseed oil generally employed in the manufacture of floor coverings or floor cloth such as linoleum. I have found that such pitches, when heated and mixed with infusorial earth or other finely divided inert substances, and preferably suitable fibrous materials, such as sawdust, or similar vegetable fiber, may be applied to canvas, or other backing to produce a floor cloth or covering having the necessary characteristics of hardness, non-conductivity, elasticity, and toughness.

To the mixture of heated pitch and infusorial earth, I find it advantageous to add a suitable fibrous material, such as powdered sawdust. The sawdust of balsawood is particularly well adapted for this purpose. Balsawood is characterized by great lightness, and very tough fiber. However, under some conditions, I find that other vegetable fibers are very well suited for this purpose. In some instances, I employ cocoanut fiber which is first prepared by cutting and grinding it to convenient sizes, for freely mixing it with heated pitch. When the pitch, infusorial earth and fibrous material have been mixed, I add such color as it is desired to impart to the mixture.

After the mixture has been prepared, it is applied under heat to canvas, or other suitable material used as a backing, and a floor cloth or covering is produced that possesses the necessary hardness, non-conductivity,

elasticity, and toughness. I find that the product so obtained compares very favorably with ordinary linoleum and is materially less costly to produce.

As an illustration of one method of producing this floor cloth, I employ 57 parts by weight of stearin pitch, palm oil pitch, or other similar pitches, or mixture of such pitches. This pitch is heated to a temperature of from 250° F. to 400° F., and while it is hot, I add thereto 8 parts by weight of infusorial earth, and 16 parts by weight of fibrous material. As stated, I employ ground sawdust for the fibrous material, preferably balsawood sawdust or cocoanut fiber. While the mixture is still hot, I add 19 parts by weight of suitable coloring material. The above proportions may be varied according to the nature of the materials used and are merely set forth as an illustration of my preferred proportions for producing a successful mixture.

Under some conditions, I find it advantageous to use a small proportion, preferably from 5 to 10 per cent. by weight of asphaltum, mineral pitch, and vegetable gums in place of a part of the residual pitch derived from the treatment of fats and oils.

While, for the purpose of illustration, I have described in detail the preferred form of my invention and the preferred proportions of materials used therein, it is to be understood that my invention is not limited thereto, but that the details of procedure and proportions of materials may be widely varied, and that known chemical equivalents of such materials may be employed, all without departing from the spirit of my invention or the scope of the subjoined claims.

What I claim is:

1. A floor covering comprising a mixture of residual pitch derived from the treatment of fats and oils, a finely divided inert substance, and fibrous material, and a suitable flexible backing for said mixture.

2. A floor covering comprising a mixture of residual pitch derived from the treatment of fats and oils, a finely divided inert substance and sawdust, and a suitable flexible backing for said mixture.

3. A floor covering comprising a mixture of residual pitch derived from the treatment of fats and oils, mineral pitch, a finely di-

vided inert substance and vegetable fiber, and a suitable flexible backing for said mixture.

4. A floor covering comprising a mixture of stearin pitch, infusorial earth, and fibrous material, and a suitable flexible backing for said mixture.

5. A floor covering comprising a mixture of a residual pitch derived from the treat-

ment of fats and oils, a finely divided inert substance, and balsawood fiber, and a suitable flexible backing for said mixture.

In testimony whereof I affix my signature in presence of two witnesses.

ALBERT C. HOLZAPFEL.

Witnesses:

CHARLES A. NANZ,  
E. H. F. MITCHELL.